

July 2, 1946.

O. SASLAW

2,403,026

SELENIUM TABLET AND METHOD OF MAKING AND APPLYING IT

Filed April 24, 1942

*Pig:1.*



*Pig:2.*



*Pig:4.*



*Pig:5.*



*Pig:5.*



INVENTOR

OTTO SASLAW

BY  
*D. J. Angus*  
ATTORNEY

## UNITED STATES PATENT OFFICE

2,403,026

SELENIUM TABLET AND METHOD OF  
MAKING AND APPLYING ITOtto Saslaw, Kearny, N. J., assignor to Federal  
Telephone & Radio Corporation, a corporation  
of Delaware

Application April 24, 1942, Serial No. 440,411

6 Claims. (Cl. 117—110)

1

This invention relates to selenium wafers or tablets and methods of making them and of applying them to a base plate to form selenium elements.

The object of this invention is to provide a simple method of making a selenium wafer in a form from which it can readily be applied to a base plate.

In the making of selenium discs heretofore it has been customary to apply amorphous selenium powder, preferably in the vitreous form, on a base plate, heat the plate to fuse the selenium, and spread the selenium over the plate while it is being fused. Considerable time has been taken in spreading the fused powder, owing in large part to the high surface tension of molten selenium and also the fact that air bubbles must be removed. The length of time required to coat the hot plate has the disadvantage that those parts of the plate which have not yet received the selenium readily oxidize which tends to injure the final product.

In accordance with my invention, I provide the selenium in a wafer or tablet form and preferably make the tablet of the proper size to cover the base plate, so that by placing the wafer or tablet on the base plate, which is heated, all parts of the surface of the base plate are simultaneously covered with the selenium and the fusing takes place simultaneously over all parts of the surface. This facilitates the application of the selenium to the plate and minimizes the undesired oxidation of part of the plate which might occur if such parts were left uncovered for a time while hot.

In the drawing:

Fig. 1 illustrates the pressure plates of a press in which the wafer may be made;

Fig. 2 is a face view of a wafer made according to this invention;

Fig. 3 is a side view of the wafer;

Fig. 4 illustrates a base plate on which the wafer has been placed; and

Fig. 5 is a cross-sectional view of the plate and wafer of Fig. 4.

According to this invention, a measured quantity of selenium, in the amount desired to be placed on the plate to be coated, is compressed between the pressure plate of a press. This is illustrated in Fig. 1 wherein the selenium in the well known black vitreous powder form is placed between the pressure heads 2 and 3 of the press, the rest of the press mechanism not being shown. The pressure heads are preferably formed with wells 4 and 5, respectively, so that heating ele-

2

ments may be placed in these wells to heat up the heads while the pressure is being applied. The actual surfaces between which the selenium wafer is to be pressed should be of a material which is not injurious to the selenium, and for this purpose mica and aluminum have been found satisfactory. The plates 6 and 7 are accordingly preferably made or faced with mica or aluminum. A pressure which I have found satisfactory is several thousand pounds per square inch and I have found 120° C. a proper temperature to use at this pressure. It will be understood that the permissible pressure and temperature can vary considerably from these particular values however. In actual practice, the amount of pressure and the temperature will bear a proper relation to the thickness of the selenium sheet which is desired, and this in turn will depend upon the amount of selenium with which it is desired to coat on the base plate. It will be found that the wafer of selenium will form quickly under the temperature and pressure, owing in large part to the cohesive properties of selenium. The thickness of the wafer will likewise depend, of course, upon the amount of the selenium powder compressed. The shape of the selenium wafer need not necessarily be circular as shown in Fig. 2, but might be made square or rectangular or some other shape, as desired, the shape being determined somewhat by the shape in which the powder is first applied between the pressure plate. For example, if a circular wafer is desired, the powder should be piled evenly in a pile between the pressure plates, so that when warmed and pressed it will spread out evenly in all directions into the circular shape. Such a circular finished tablet is shown in Figs. 2 and 3, which will be removed from the press as a solid, unbending wafer.

40 The application of this wafer to a base plate is illustrated in Figs. 4 and 5, wherein the wafer 8 is shown placed upon the base plate 9 which will ordinarily have in it a central hole 10. The base plate should be heated up to a temperature above the melting point of the selenium to melt the wafer. The melting will occur uniformly throughout the surface of the plate and will be rapid enough so that very little oxidation will form on the plate prior to the melting and fusing of the selenium. As is well known, if such a molten layer of selenium be allowed to cool down to about room temperature it solidifies, forming a vitreous non metallic coating, which could be converted, if desired, to the metallic

form by heat treating at a temperature somewhat below the melting point of selenium.

In this fusing operation a slight amount of touching up of the molten selenium to the plate may be required to compensate for the surface tension shrinkage of the selenium, in order to obtain a uniform coverage and fusing.

The use of such a selenium wafer and the method of application to the base plate is advantageous both from the point of view of simplicity and of advantageous effect on the plate. The method is simple as the coating operation requires less work than in the heretofore used method of puddling and spreading the selenium fused from powder over the surface of the base plate. The application of the wafer to the base plate allows substantially all of the surface of the base plate to come immediately into contact with the selenium, so that excessive oxidation of any part of the hot base plate surface caused by exposure to heat and air before it is completely selenium coated, is completely eliminated.

An alternative method of making the selenium wafer or tablet is to convert the tablet of vitreous amorphous selenium, taken from the press, into the gray metallic state before applying it to the base plate. This may be done by taking the vitreous tablet shown in Figs. 2 and 3 and heating it at a temperature of from 170° C. to 217° C. A temperature of 200° C. is found highly advantageous. This high temperature heating should be continued until the black color of the vitreous form of tablet is converted to the gray metallic color. It has been found that the gray metallic tablet covers the base plate surface more evenly than does the vitreous type of tablet upon melting.

If the tablet is made slightly oversize with respect to the base plate, it will be found that upon melting, the tablet will assume almost the exact shape of the base plate contact surface. Hence, it is advantageous to make the tablet somewhat oversize if complete coverage is desired. It will also be found that the surface tension of the selenium will act to cause it to uncover the central hole 10 which is usually pressed in the base plate or cathode 9 of the selenium rectifier. The reason for this is that the shrinkage of the tablet during the heating and fusing at the position over the hole where it is unattached to the base plate causes a corresponding hole to open up through the selenium as the selenium over the hole is drawn by its surface tension toward the base plate.

It should be understood that the invention is not necessarily limited to the making or use of vitreous or metallic selenium wafers, as it is possible to make the wafers of red amorphous selenium powder in substantially the same way as in the case of the vitreous wafers. The use of the

vitreous form instead of red form is usually preferable for use in rectifiers, as the vitreous form has been found to give the better results.

References herein to selenium elements are intended to cover selenium rectifiers and selenium photo-electric cells.

What is claimed is:

1. In the manufacture of selenium elements, the method of coating a base plate with selenium, which comprises completely covering the surface of the base plate to be coated with a wafer of compressed selenium powder, and heating the plate to a temperature sufficient to fuse the selenium to the surface.

2. In the manufacture of selenium elements, the method of coating a base plate with selenium, which comprises completely covering the surface of the base plate to be coated with a wafer of compressed selenium powder, and then heating the plate to a temperature above the melting point of selenium to melt the wafer and fuse the selenium to the surface.

3. The method of making a selenium element, which comprises completely covering the surface of a base plate with a thin cohesive selenium wafer, and heating the base plate to melt the selenium.

4. The method of making a selenium element, which comprises compressing amorphous selenium powder under high pressure and at an elevated temperature in the general order of about 120° C. to form a cohesive wafer, then completely covering with said wafer the surface of a base plate to be coated with the selenium, and heating the base plate to fuse the selenium to the surface.

5. The method of making a selenium element, which comprises making a wafer by compressing selenium powder under a pressure of the general order of several thousand pounds per square inch at a temperature in the general neighborhood of about 120° C., then completely covering by said wafer the surface of a base plate to be coated with the selenium, and then fusing the wafer to said surface by heating the base plate to the fusing point of selenium.

6. The method of making a selenium element, which comprises compressing amorphous selenium powder at a temperature in the general neighborhood of about 120° C. and a pressure of the general order of several thousand pounds per square inch, to form a selenium wafer, then converting the wafer to the metallic form by heating it at a temperature of the general order of about 170° C. to 217° C., then completely covering by the wafer the surface of a base plate to be coated, and then fusing the metallic wafer to the plate by heating the plate to the fusing point of selenium.

OTTO SASLAW.